

Patented Dec. 31, 1946

2,413,501

# UNITED STATES PATENT OFFICE

2,413,501

## ARTIFICIAL FIBERS FROM GLOBULAR AND FIBROUS PROTEINS

Oskar Huppert, New York, N. Y.

No Drawing. Application February 12, 1945,  
Serial No. 577,593

3 Claims. (CL 260—119)

1

This application is a continuation in part of the one filed on May 24, 1944, bearing Serial No. 537,190, now U. S. Patent 2,384,421. My invention deals with fibers made from proteins. The object of this invention is to produce dispersions of proteins, which can be used to make fibers, which have strength, water resistance, flexibility and softness and are valuable as fibers.

A further object resides in processes for making these dispersions. Other objects of the invention will appear as the description proceeds.

These objects are accomplished by the following invention in which dispersions of pseudothiobiohydantoin-protein salts of alkyl-benzene-sulfonic acid of the general formula as follows:



wherein protein'-NH<sub>2</sub> denotes protein, are used to produce artificial fibers from globular and fibrous proteins by spinning and stretching, hardening, pre and after treatment methods with various modifying agents already known to the art.

All proteins can be transformed into pseudothiobiohydantoin-proteins by a process described in U. S. Patent No. 2,343,012, and in U. S. Patent No. 2,364,034.

I have discovered, that the reaction takes place also in presence of ammonia, where a protein is used which would be precipitated on the acid side of its isoelectric point. According to this invention fibers may be prepared either from an ammonia alkaline-aqueous solution where a protein is used as for instance casein, soybean or peanut protein, egg albumin, reduced chicken feather keratin or from an alcoholic-aqueous solution where a protein is used as for instance zein, gliadin or other prolamines, protamines. The present ideas of the structural units of natural fibers as chain molecules developed by Astbury, Mark and Meyer and others are not able to disclose the structural difference of globular and fibrous proteins. My work to establish the structure of the proteins starts from early statements, published in "Konstitution und Konfiguration der Eiweiß-stoffe, Wien-Liepzig, 1928" and is used in the present application. Textile fibers should have strength and flexibility. Globular (sphero) proteins as such are not fit for preparing fibers, only fibrillar (linear) proteins are capable of forming fibers which in certain circumstances are sufficiently tough and elastic to possess some technical interest. These both classes of natural high polymers are different in kind of their structural units. Natural fibers consist of open, long polypeptide chains, which may be completely extended (beta-keratin type) or coiled (alpha-keratin type) or super-

2

contracted. More or less cross linked by means of secondary valences through polar groups, salt linkages they form with their side chains a coplanar three dimensional arrangement. Because of free rotation around single bonds the structural units of natural fibers are capable of being oriented and to form crystal lattices which favors fiber strength and flexibility, if there is not completely cross linking.

10 The current view of globular protein according X-ray analysis is that crystalline globular proteins have a compact structure, that the very regularly built molecules contain a considerable amount of water. The very highly ordered structure, revealed by X-ray photographs of protein crystals, discloses, that the chains of the globular proteins must be built into a very systematic pattern of folds. On treatment with denaturating agents a breakdown of this special ordered structure occurs and the resulting products aggregate on coagulation into fibrous bundles which have been shown by X-ray study to be of the beta keratin type. An intimate relation between the fibrous and the globular proteins is therefore indicated. Therefore a transformation of globular proteins in fibrous proteins should be possible. However, neither the cyclol hypothesis of D. M. Wrinch (1936) nor the models of Huggins (1940) have shown wherein the special configuration of the chains of the globular proteins consists and the X-ray diffraction patterns of the globular proteins are still not sufficiently advanced.

15 Based on the reaction of carbon disulfide, and proteins, protein hydrolysates, alpha amino acids, U. S. Patent 2,112,210 and on the physiological and physical-biochemical reactions of natural, native proteins in the living organism I conceived in my publication "Das Protein" Wien, 1933, the 20 "Proteyl-theory." Accordingly all globular proteins are built up on the same general pattern from normal proteyls,



25 or from pseudo-proteyls,



30 which six of each are in space configurated under an angle of 60 degrees in the boat type, representing the isomeres of the elementary units of the protein. The elementary unit exists in three stereoisomeric forms. The normal form showing relations with dioxopiperazines, oxazolines, triazoles, acetaldehyde, the pseudo form with hexoses, hexosamines, glucose, the purin form 35 with beta ketonic acids, acetone, pyridine, purin and pyrimidine glucosides, purin bases such as

adenine, guanine and pyrimidine bases, such as cytosine and uracil, the combined normal-pseudo form with isoprene, phytol, terpene derivatives and carotenoides. The following formulas give the structure and configuration of the elementary units of the protein:

ISOMERES OF THE ELEMENTARY UNITS OF THE PROTEIN



Two such normal proteyls, belonging to two different elementary units, would formally result by condensation of two mol alpha amino acids in the "zwitter ion form" as follows:



showing the peptide-betain linkage encircled.

This network of proteyls changes in a bundle of polypeptide chains resulting from the conversion of the peptide-betain linkage in a peptide-linkage as follows:



and thus effecting the transformation of the globular proteins in the fibrous proteins.

At last the difference of globular and fibrous proteins consists in the deposition of water (internal hydration) between the proteyls girders of the individual elementary units. According the proteyl theory in contrast to Emil Fischer's conception proteins are not built up from amino acids having the structure,  $(-\text{CO}-\text{CH}(\text{R})-\text{NH}-)_n$ , but from hydrated proteyls having the structure



Any non-proteolytic modification of the unique structure of a native protein resulting under the influence of denaturating agents is a step in the continuous line of a dynamic process leading from the very systematic and specific pattern of the six in space configurated proteyls under breakdown of the proteyl-girder to unfolded polypeptide chains of the beta keratin type with the intermediate stages of super contracted and coiled polypeptide chains.

Associating water as well on the polar, hydrophilic groups of their side chains (external hydration) as on the oxygen atoms of the girder, the hydration degree of the proteins turns out to be decisive for the osmotic pressure and viscosities of the protein solutions while the denaturation-kinetic of the proteins becomes the determinative factor for their ability to be spun in fibers.

Solutions containing salts of pseudothiohydantoin-protein (fibrous and globular), with alkyl-benzene sulfonic acids can be used to precipitate the synthetic protein in a coagulating bath into a plastic state, favorable for drawing into fibers. On the alkaline side of the isoelectric point anions of the alkyl-benzene sulfonic acid exert an influence conducive to the transformation of the globular proteins in fibrous proteins by drawing the fibers over 300%.

The following examples are illustrative for all proteins and will serve to show certain specific details of the invention, however, it is to be understood that the specific details as set forth in the examples are not to be considered as limitative of the invention.

Example 1

Casein fibers are spun from a solution having the following composition: 110 grams of casein are soaked in 555 cc. of water at 24° C. containing 9.4 g. monochloracetic acid, 7.6 g. ammonium thiocyanate, 8.1 g. p-toluene sulfonic acid cryst. and 21 cc. concentrated ammonium hydroxide with stirring. After three hours the dispersion is heated to 45° C. and the ripened and deaerated solution is forced through a spinneret of forty holes and of a diameter of 0.004 inch into a coagulating bath having the composition: water 100 cc., conc. sulfuric acid 15 g., anhydrous sodium sulfate 20 g., aluminum sulfate (hydrate) 10 g. The coagulated fibers are afterwards stretched in

## 5

a bath containing 15% sodium chloride at a temperature over 50° C. The fibers are now washed and dried without tension.

## Example 2

Soya bean protein fibers are spun from a solution having the following composition:

|                                 |    |     |
|---------------------------------|----|-----|
| Water                           | cc | 806 |
| Monochloracetic acid            | g  | 15  |
| Ammoniumthiocyanate             | g  | 12  |
| p-Toluene sulfonic acid cryst.  | g  | 13  |
| Concentrated ammonium hydroxide | cc | 33  |
| Alpha soya bean protein         | g  | 180 |

After soaking the protein for 30 minutes at a 15 temperature of 45° C. the dispersion is warmed to 65° C. and mixed under stirring. The spinning solution after permitting to mature is then forced under stretching through a spinneret into a coagulating bath as follows:

|                |          |    |
|----------------|----------|----|
| Water          | per cent | 55 |
| Acid sulfuric  | do       | 25 |
| Sodium sulfate | do       | 20 |
| Temperature    | ° C.     | 45 |

The fibers are afterwards thoroughly washed and dried without tension, using a current of air, after they were hardened in a bath as follows:

|                 |    |    |
|-----------------|----|----|
| Water           | 95 | 30 |
| Formaldehyde    | 4  |    |
| Sodium chloride | 1  |    |

## Example 3

Fibers from zein are prepared by extrusion of 35 a solution, which is obtained by dissolving in a mixture of 300 cc. of denatured alcohol and 36 cc. of water 1.8 g. monochloracetic acid, 1.35 g. ammoniumthiocyanate and 1.5 g. p-toluene-sulfonic acid cryst. and after addition of 90 g. of zein 40 by heating under stirring for a half hour. The spinneret used is the usual forty holes viscose spinneret and the coagulating bath consists of 5% aluminum sulfate. After washing the filaments are stretched in warm water and then passed into 45 cold water and treated with 6% formaldehyde so-

lution. The fibers are washed with cold water again and dried.

Having now particularly described and ascertained the nature of my said invention, I declare that what I claim is:

1. As a new article of manufacture, a fiber consisting of an alkyl-benzene-sulfonic acid salt of a pseudothiohydantoin, substituted in position 3 by a protein radical selected from the group consisting of phospho-proteins, globulins and prolamines, having the formula:



wherein protein' represents the residue of a protein molecule after removal of NH<sub>2</sub>— therefrom.

2. As a new article of manufacture, a fiber consisting of a para toluene-sulfonic acid salt of a pseudothiohydantoin, substituted in position 3 by a protein radical selected from the group of phosphoproteins, globulins and prolamines, having the formula:



wherein protein' represents the residue of a protein molecule after removal of NH<sub>2</sub>— therefrom.

3. As a new article of manufacture, a fiber consisting of a para toluene-sulfonic acid salt of a pseudothiohydantoin, substituted in position 3 by the radical of casein, having the formula:



wherein casein' represents the residue of a casein molecule after removal of NH<sub>2</sub>— therefrom.

OSKAR HUPPERT.